

# UNITED STATES PATENT OFFICE.

JOSEPH A. DIETZ, OF ST. MARY'S, PENNSYLVANIA, ASSIGNOR OF ONE-HALF  
TO ERNEST J. WIMMER, OF SAME PLACE.

## PROCESS OF MAKING LEATHER WATER-PROOF.

SPECIFICATION forming part of Letters Patent No. 334,518, dated January 19, 1886.

Application filed December 29, 1884. Serial No. 151,517. (No specimens.)

*To all whom it may concern:*

Be it known that I, JOSEPH A. DIETZ, a citizen of the United States of America, residing at St. Mary's, in the county of Elk and State 5 of Pennsylvania, have invented a new and useful composition of matter to be used upon tanned sole-leather, upper-leather, calf-skin, and all other kinds of leather, and method of applying the same, for the purpose of making 10 said leathers water-proof, and also more pliable and durable, of which the following is a specification.

My composition consists of the following ingredients combined in the proportions stated 15 and used as stated, viz: Cold water. Soak the leather therein thoroughly. After the leather is half-dry apply the following with a sponge: sugar of lead, one ounce; hot water, one gallon. Then next apply the following with a 20 different sponge: alum, (common potash-alum,) two pounds; hot water, two gallons. These amounts will suffice for half a dozen hides. Said ingredients (sugar of lead and hot water) are to be thoroughly mixed by agitation, as also are the alum and hot water.

In using the above-named composition the 25 hides should be first well scoured and half-dried. The solutions must be applied upon both sides of the hides, and can be applied 30 immediately to rough hides (half-dried) or after the hides are finished.

I am aware that compositions exist upon

which Letters Patent have been issued and granted, which are used for the same purpose, viz: No. 131,563, to P. V. Roudiez on September 24, 1872, and No. 250,874, to Valentine Belikan on December 13, 1881; but I am not aware that all of the ingredients of my composition, in the proportions stated, have been used as above stated and applied, as stated 40 herein.

What I claim, and desire to secure by Letters Patent of the United States, is—

1. The within method of treating leather and hides and the like to render them water-repellent and pliable, consisting in applying water thereto, then partially drying the same, then applying a solution of sugar of lead and hot water, and subsequently applying a solution of alum and hot water, substantially as described.

2. The within compound for treating leather and hides and the like to render them water-repellent and pliable, composed of two solutions, one being hot water one gallon and sugar of lead one ounce, and the other hot water two gallons and alum two pounds, to be used in the order named, substantially as described.

JOSEPH A. DIETZ.

Witnesses:

GEORGE AUMAN,  
GEO. ED. WEIS.